



US005273669A

**United States Patent** [19]

Schumacher et al.

[11] **Patent Number:** 5,273,669[45] **Date of Patent:** Dec. 28, 1993[54] **LUBRICANT COMPOSITION**

[75] Inventors: Rolf Schumacher; Samuel Evans; Paul Dubs, all of Marly, Switzerland

[73] Assignee: Ciba-Geigy Corporation, Ardsley, N.Y.

[21] Appl. No.: 951,377

[22] Filed: Sep. 25, 1992

**Related U.S. Application Data**

[60] Continuation of Ser. No. 771,085, Oct. 2, 1991, abandoned, which is a division of Ser. No. 380,563, Jul. 13, 1989, Pat. No. 5,073,278.

[30] **Foreign Application Priority Data**

Jul. 18, 1988 [CH] Switzerland 2737/88

[51] Int. Cl.<sup>5</sup> C10M 135/36; C10M 133/40

[52] U.S. Cl. 252/47.5; 252/47; 252/50; 252/51.5 R

[58] **Field of Search** 252/47.5, 47, 50, 51.5 R[56] **References Cited****U.S. PATENT DOCUMENTS**

- 3,218,256 11/1965 Edwards 252/47  
 3,480,635 11/1969 Altwicker 252/50  
 3,523,910 8/1970 Randell 252/47  
 3,535,243 10/1970 Chao et al. 252/50  
 3,539,515 11/1970 McCabe 252/47  
 3,689,484 9/1972 Spilners 252/47  
 3,773,665 11/1973 Braid 252/50  
 3,822,209 7/1974 Knapp et al. 546/184  
 3,844,958 10/1974 Anderson et al. 252/50  
 4,370,246 1/1983 de Vries et al. 252/50  
 4,461,898 7/1984 Meier et al. 546/188  
 4,525,503 6/1985 Cantatore 546/188  
 4,540,732 9/1985 Spivack et al. 524/289  
 4,601,839 7/1986 Lai 252/51.5 A  
 4,691,015 9/1987 Behrens et al. 546/188  
 4,692,258 9/1987 Rasberger et al. 252/50  
 4,695,599 9/1987 Cantatore 546/188

- 4,824,601 4/1989 Franklin 252/50  
 5,035,817 7/1991 Salomon 252/47.5  
 5,073,278 12/1991 Schumacher et al. 252/47.5

**FOREIGN PATENT DOCUMENTS**

- 0049133 4/1982 European Pat. Off. .  
 0059168 9/1982 European Pat. Off. .  
 0239536 9/1987 European Pat. Off. .  
 0286595 10/1988 European Pat. Off. .  
 WO8802007 3/1988 PCT Int'l Appl. .  
 0933505 9/1963 United Kingdom .  
 1090688 12/1967 United Kingdom .  
 1140089 1/1969 United Kingdom .  
 1347141 2/1974 United Kingdom .  
 1438482 6/1976 United Kingdom .

*Primary Examiner*—Ellen M. McAvoy  
*Attorney, Agent, or Firm*—Luther A. R. Hall

[57] **ABSTRACT**

A lubricant based on a mineral or synthetic oil is stabilized against oxidative degradation by the addition of a mixture comprising at least one specified aromatic amine of the formula I or II



and at least one sterically hindered amine. The lubricant may contain other antioxidants or other additives. It is preferably used as motor oil.

**8 Claims, No Drawings**

## LUBRICANT COMPOSITION

This is a continuation of application Ser. No. 07/771,085, filed on Oct. 2, 1991, now abandoned, which is a divisional of application Ser. No. 07/380,563, filed Jul. 13, 1989, now U.S. Pat. No. 5,073,278, issued on Dec. 17, 1991.

The present invention relates to lubricant compositions which are stabilized against oxidative degradation. The stabilization is carried out by the addition of at least two specific additives.

It is known and customary to add additives to lubricants based on mineral or synthetic oils in order to improve their performance characteristics. Additives against oxidative degradation of the lubricants, the so-called antioxidants, are of particular importance. Oxidative degradation of lubricants plays a significant role especially in motor oils because of the high temperatures prevailing in the combustion chambers of the engines and the presence, in addition to oxygen, of oxides of nitrogen ( $\text{NO}_x$ ) which act as oxidation catalysts.

## SUMMARY OF THE INVENTION

Aromatic amines, for example alkylated diphenylamines or alkylated phenothiazines, are used inter alia as antioxidants for lubricants. EP-A-149,422 or GB-A-1,090,688, for example, disclose such amines. The use of such aromatic amines in combination with other antioxidants, for example with triarylphosphites, thiadipropionates or phenolic antioxidants, is also known, for example from EP-A-49,133.

We have found that a combination of aromatic amines with sterically hindered amines is a highly suitable antioxidant for lubricants.

The invention provides a lubricant composition which comprises

(A) a mineral or a synthetic base oil or a mixture of such oils,

(B) at least one aromatic amine of the formula I or II,



in which  $\text{R}^1$  is  $\text{C}_1\text{-C}_{18}\text{alkyl}$ ,  $\text{C}_7\text{-C}_9\text{phenylalkyl}$ ,  $\text{C}_5\text{-C}_{12}\text{cycloalkyl}$ , phenyl,  $\text{C}_7\text{-C}_{18}\text{alkylphenyl}$ ,  $\text{C}_7\text{-C}_{18}\text{alkoxyphenyl}$  or naphthyl,  $\text{R}^2$  is phenyl,  $\text{C}_7\text{-C}_{18}\text{alkylphenyl}$ ,  $\text{C}_7\text{-C}_{18}\text{alkoxyphenyl}$  or naphthyl,  $\text{R}^3$  is hydrogen,  $\text{C}_1\text{-C}_{12}\text{alkyl}$ , benzyl, allyl, methallyl, phenyl or a group  $-\text{CH}_2\text{SR}^4$ ,  $\text{R}^4$  is  $\text{C}_4\text{-C}_{18}\text{alkyl}$ ,  $-\text{CH}_2\text{COO}(\text{C}_4\text{-C}_{18}\text{alkyl})$  or  $-\text{CH}_2\text{CH}_2\text{COO}(\text{C}_4\text{-C}_{18}\text{alkyl})$ , and  $\text{R}^5$  and  $\text{R}^6$  independently of one another are H,  $\text{C}_1\text{-C}_{18}\text{alkyl}$  or  $\text{C}_7\text{-C}_9\text{phenylalkyl}$ , and

(C) at least one sterically hindered amine.

## DETAILED DESCRIPTION OF THE INVENTION

As  $\text{C}_1\text{-C}_{12}\text{alkyl}$ ,  $\text{R}^3$  may be linear or branched alkyl and may be, for example, methyl, ethyl, propyl, butyl, pentyl, hexyl, octyl, nonyl, decyl or dodecyl. As  $\text{C}_1\text{-C}_{18}\text{alkyl}$ ,  $\text{R}^1$ ,  $\text{R}^5$  and  $\text{R}^6$  may in addition also be, for example, tetradecyl, pentadecyl, hexadecyl or octadecyl. As  $\text{C}_4\text{-C}_{18}\text{alkyl}$ ,  $\text{R}^4$  may also be, for example, n-butyl, tert-butyl, n-hexyl, tert-octyl, n-dodecyl or octadecyl.

As  $\text{C}_7\text{-C}_9\text{phenylalkyl}$ ,  $\text{R}^1$ ,  $\text{R}^5$  and  $\text{R}^6$  may be, for example, benzyl, 2-phenylethyl,  $\alpha$ -methylbenzyl, 2-phenylpropyl or  $\alpha,\alpha$ -dimethylbenzyl.

As  $\text{C}_7\text{-C}_{18}\text{alkylphenyl}$ ,  $\text{R}^1$  and  $\text{R}^2$  may have linear or branched alkyl groups. Examples are tolyl, ethylphenyl, isopropylphenyl, tert-butylphenyl, sec-pentylphenyl, n-hexylphenyl, tert-octylphenyl, iso-nonylphenyl or n-dodecylphenyl.  $\text{R}^1$  and  $\text{R}^2$  may also be mixtures of alkylphenyl groups, such as those produced in industrial alkylations of diphenylamine with olefins. The alkyl group is preferably in the para position of the aromatic amine.

As the component (B), a compound of the formula I or II is preferably used in which  $\text{R}^1$  is  $\text{C}_1\text{-C}_{18}\text{alkyl}$ ,  $\text{C}_7\text{-C}_9\text{phenylalkyl}$ , cyclohexyl, phenyl,  $\text{C}_{10}\text{-C}_{18}\text{alkylphenyl}$  or naphthyl,  $\text{R}^2$  is  $\text{C}_{10}\text{-C}_{18}\text{alkylphenyl}$  or phenyl,  $\text{R}^3$  is hydrogen,  $\text{C}_1\text{-C}_{18}\text{alkyl}$ , benzyl, allyl or a group  $-\text{CH}_2\text{SR}^4$ ,  $\text{R}^4$  is  $\text{C}_8\text{-C}_{18}\text{alkyl}$  or  $-\text{CH}_2\text{COO}(\text{C}_8\text{-C}_{18}\text{alkyl})$ , and  $\text{R}^5$  and  $\text{R}^6$  independently of one another are H,  $\text{C}_1\text{-C}_{12}\text{alkyl}$  or  $\text{C}_7\text{-C}_9\text{phenylalkyl}$ .

Of the compounds of the formula I those are particularly preferred in which  $\text{R}^1$  and  $\text{R}^2$  independently of one another are phenyl or  $\text{C}_{10}\text{-C}_{18}\text{alkylphenyl}$  and  $\text{R}^3$  is hydrogen.

Of the compounds of the formula II those are particularly preferred in which  $\text{R}^3$  is hydrogen and  $\text{R}^5$  and  $\text{R}^6$  independently of one another are H or  $\text{C}_4\text{-C}_{12}\text{alkyl}$ .

Examples of compounds of the formula I are:

diphenylamine,

N-allyldiphenylamine

4-isopropoxydiphenylamine

N-phenyl-1-naphthylamine

N-phenyl-2-naphthylamine

di-4-methoxydiphenylamine

d-[4-(1,3-dimethylbutyl)phenyl]amine

di-[4-(1,1,3,3-tetramethylbutyl)phenyl]amine

tert-octylated N-phenyl-1-naphthylamine

industrial mixtures obtained by reacting diphenylamine with diisobutylene (mono-, di- and trialkylated tert-butyl- and tert-octyldiphenylamine)

phenothiazine

N-allylphenothiazine

3,7-di-tert-octylphenothiazine

industrial mixtures obtained by reacting phenothiazine with diisobutylene

Particularly preferred component (B) is 4,4'-di-tert-octyldiphenylamine or 3,7-di-tert-octylphenothiazine or an industrial mixture obtained by reacting diphenylamine with diisobutylene, particularly a mixture which contains the following components:

- not more than 5% by weight of diphenylamine,
- 8-15% by weight of 4-tert-butylidiphenylamine,
- 24-32% by weight of 4-tert-octyldiphenylamine, 4,4'-di-tert-butylidiphenylamine and 2,4,4'-tri-tert-butylidiphenylamine,
- 23-34% by weight of 4-tert-butyl-4'-tert-octyldiphenylamine, 2,2'- and 3,3'-di-tert-octyldiphenylamine.

mine and 2,4-di-tert-butyl-4'-tert-octyl-diphenylamine,  
e) 21-34% by weight of 4,4'-di-tert-octyl diphenylamine and 2,4-di-tert-octyl-4'-tert-butyl diphenylamine.

The component (C) may be any cyclic or acyclic sterically hindered amine. The preferred component (C) is a compound which contains at least one group of the formula III



in which R is hydrogen or methyl. R as hydrogen is preferred. The compounds in question are derivatives of polyalkylpiperidines, particularly of 2,2,6,6-tetramethylpiperidine. These polyalkylpiperidines preferably carry one or two polar substituents or a polar spiro ring system in the 4-position.

The following classes of polyalkylpiperidines are particularly important:

a) compounds of the formula IV



in which n is an integer of 1 to 4, preferably 1 or 2, R is hydrogen or methyl, R11 is hydrogen, oxy, hydroxyl, C1-C12alkyl, C3-C8alkenyl, C3-C8alkynyl, C7-C12aralkyl, C1-C18alkoxy, C5-C8cycloalkoxy, C7-C9phenylalkoxy, C1-C8alkanoyl, C3-C5alkenoyl, C1-C18alkanoyloxy, benzyl, glycidyl or a group —CH2C—H(OH)—Z, in which Z is hydrogen, methyl or phenyl, R11 being preferably H, C1-C4alkyl, allyl, benzyl, acetyl or acryloyl and R12 being, when n is 1, hydrogen, C1-C18alkyl which is uninterrupted or interrupted by one or more oxygen atoms, cyanoethyl, benzyl, glycidyl, a monobasic radical of an aliphatic, cycloaliphatic, araliphatic, unsaturated or aromatic carboxylic acid, carbamic acid or a phosphorus-containing acid or a monovalent silyl radical, preferably a radical of an aliphatic carboxylic acid having 2 to 18 carbon atoms, of a cycloaliphatic carboxylic acid having 7 to 15 carbon atoms, of an  $\alpha,\beta$ -unsaturated carboxylic acid having 3 to 5 carbon atoms or of an aromatic carboxylic acid having 7 to 15 carbon atoms, R12 being, when n is 2, C1-C12alkylene, C4-C12alkenylene, xylylene, a dibasic radical of an aliphatic, cycloaliphatic, araliphatic or aromatic dicarboxylic acid, dicarbamic acid or a phosphorus-containing acid or a divalent silyl radical, preferably a radical of an aliphatic dicarboxylic acid having 2 to 36 carbon atoms, a cycloaliphatic or aromatic dicarboxylic acid having 8 to 14 carbon atoms or an aliphatic, cycloaliphatic or aromatic dicarbamic acid having 8 to 14 carbon atoms, R12 being, when n is 3, a tribasic radical of an aliphatic, cycloaliphatic or aromatic tricarboxylic acid, an aromatic tricarbamic acid or a phosphorus-containing acid or a trivalent silyl radi-

cal, and R12 being, when n is 4, a tetrabasic radical of an aliphatic, cycloaliphatic or aromatic tetracarboxylic acid.

Any C1-C12alkyl substituents present are, for example, methyl, ethyl, n-propyl, n-butyl, sec-butyl, tert-butyl, n-hexyl, n-octyl, 2-ethylhexyl, n-nonyl, n-decyl, n-undecyl or n-dodecyl.

As C1-C18alkyl, R11 or R12 may be, for example, the above groups and additionally, for example, n-tridecyl, n-tetradecyl, n-hexadecyl or n-octadecyl.

As C3-C8alkenyl, R11 is, for example, 1-propenyl, allyl, methallyl, 2-butenyl, 2-pentenyl, 2-hexenyl, 2-octenyl and 4-tert-butyl-2-but enyl.

As C3-C8alkynyl, R11 is preferably propargyl.

As C7-C12aralkyl, R11 is particularly phenethyl and above all benzyl.

As C1-C8alkanoyl, R11 is, for example, formyl, propionyl, butyryl, octanoyl, but preferably acetyl; and as C3-C8alkenoyl, R11 is particularly acryloyl.

As a monobasic radical of a carboxylic acid, R12 is a radical, for example, of acetic acid, caproic acid, stearic acid, acrylic acid, methacrylic acid, benzoic acid or  $\beta$ -(3,5-di-tert-butyl-4-hydroxyphenyl)-propionic acid.

As a dibasic radical of a dicarboxylic acid, R12 is a radical, for example, of malonic acid, succinic acid, glutaric acid, adipic acid, suberic acid, sebatic acid, maleic acid, itaconic acid, phthalic acid, dibutylmalonic acid, dibenzylmalonic acid, butyl(3,5-di-tert-butyl-4-hydroxybenzyl)malonic acid or bicycloheptenedicarboxylic acid.

As a tribasic radical of a tricarboxylic acid, R12 is a radical, for example, of trimellitic acid, citric acid or nitrilotriacetic acid.

As a tetrabasic radical of a tetracarboxylic acid, R12 is the tetrabasic radical, for example, of butane-1,2,3,4-tetracarboxylic acid or of pyromellitic acid.

As a dibasic radical of a dicarbamic acid, R12 is a radical, for example, of hexamethylenedicarbamic acid or 2,4-toluenedicarbamic acid.

Preferred compounds of the formula IV are those in which R is hydrogen, R11 is hydrogen or methyl, n is 2 and R12 is the diacyl radical of an aliphatic dicarboxylic acid having 4 to 12 carbon atoms.

Examples of polyalkylpiperidine compounds of this class are the following compounds:

- 1) 4-hydroxy-2,2,6,6-tetramethylpiperidine
- 2) 1-allyl-4-hydroxy-2,2,6,6-tetramethylpiperidine
- 3) 1-benzyl-4-hydroxy-2,2,6,6-tetramethylpiperidine
- 4) 1-(4-tert-butyl-2-but enyl)-4-hydroxy-2,2,6,6-tetramethylpiperidine
- 5) 4-stearoyloxy-2,2,6,6-tetramethylpiperidine
- 6) 1-ethyl-4-salicyloyloxy-2,2,6,6-tetramethylpiperidine
- 7) 4-methacryloyloxy-1,2,2,6,6-pentamethylpiperidine
- 8) 1,2,2,6,6-pentamethylpiperidin-4-yl-(3,5-di-tert-butyl-4-hydroxyphenyl) propionate
- 9) di-(1-benzyl-2,2,6,6-tetramethylpiperidin-4-yl) maleate
- 10) di-(2,2,6,6-tetramethylpiperidin-4-yl) succinate
- 11) di-(2,2,6,6-tetramethylpiperidin-4-yl) glutarate
- 12) di-(2,2,6,6-tetramethylpiperidin-4-yl) adipate
- 13) di-(2,2,6,6-tetramethylpiperidin-4-yl) sebacate
- 14) di-(1,2,2,6,6-pentamethylpiperidin-4-yl) sebacate
- 15) di-(1,2,3,6-tetramethyl-2,6-diethylpiperidin-4-yl) sebacate
- 16) di-(1-allyl-2,2,6,6-tetramethylpiperidin-4-yl) phthalate

- 17) 1-hydroxy-4--cyanoethoxy-2,2,6,6-tetramethylpiperidine  
 18) 1-acetyl-2,2,6,6-tetramethylpiperidin-4-yl acetate  
 19) tri-(2,2,6,6-tetramethylpiperidin-4-yl) trimellitate  
 20) 1-acryloyl-4-benzyloxy-2,2,6,6-tetramethylpiperidine  
 21) di-(2,2,6,6-tetramethylpiperidin-4-yl) diethylmalonate  
 22) di-(1,2,2,6,6-pentamethylpiperidin-4-yl) dibutylmalonate  
 23) di-(1,2,2,6,6-pentamethylpiperidin-4-yl) butyl-(3,5-di-tert-butyl-4-hydroxybenzyl) malonate  
 24) di(1-octyloxy-2,2,6,6-tetramethylpiperidin-4-yl) sebacate  
 25) di(1-cyclohexyloxy-2,2,6,6-tetramethylpiperidin-4-yl) sebacate  
 26) hexane-1',6'-bis(4-carbamoyloxy-1-n-butyl-2,2,6,6-tetramethylpiperidine)  
 27) toluene-2',4'-bis(4-carbamoyloxy-1-n-propyl-2,2,6,6-tetramethylpiperidine)  
 28) dimethyl-bis(2,2,6,6-tetramethylpiperidin-4-oxy)isilane  
 29) phenyl-tris(2,2,6,6-tetramethylpiperidin-4-oxy)isilane  
 30) tris(1-propyl-2,2,6,6-tetramethylpiperidin-4-yl) phosphite  
 31) tris(1-propyl-2,2,6,6-tetramethylpiperidin-4-yl) phosphate  
 32) phenyl[bis-(1,2,2,6,6-pentamethylpiperidin-4-yl)] phosphonate  
 33) 4-hydroxy-1,2,2,6,6-pentamethylpiperidine  
 34) 4-hydroxy-N-hydroxyethyl-2,2,6,6-tetramethylpiperidine  
 35) 4-hydroxy-N-(2-hydroxypropyl)-2,2,6,6-tetramethylpiperidine  
 36) 1-glycidyl-4-hydroxy-2,2,6,6-tetramethylpiperidine  
 b) compounds of the formula (V)



in which n is the integer 1 or 2, R and R<sup>11</sup> have the meaning defined in a), R<sup>13</sup> is hydrogen, C<sub>1</sub>-C<sub>12</sub>alkyl, C<sub>2</sub>-C<sub>3</sub>hydroxyalkyl, C<sub>5</sub>-C<sub>7</sub>cycloalkyl, C<sub>7</sub>-C<sub>8</sub>aralkyl, C<sub>2</sub>-C<sub>18</sub>alkanoyl, C<sub>3</sub>-C<sub>5</sub>alkenoyl, benzoyl or a group of the formula



and when n is 1, R<sup>14</sup> is hydrogen, C<sub>1</sub>-C<sub>12</sub>alkyl, C<sub>3</sub>-C<sub>5</sub>alkenyl, C<sub>5</sub>-C<sub>7</sub>cycloalkyl, C<sub>1</sub>-C<sub>4</sub>alkyl substituted by a hydroxyl, cyano, alkoxy carbonyl or carbamide group, glycidyl, a group of the formula —CH<sub>2</sub>—CH(OH)—Z or the formula —CONH—Z, in which Z is hydrogen, methyl or phenyl; when n is 2, R<sup>14</sup> is C<sub>2</sub>-C<sub>12</sub>alkylene,

C<sub>6</sub>-C<sub>12</sub>arylene, xylylene, a —CH<sub>2</sub>—CH(OH)—CH<sub>2</sub>— group or a —CH<sub>2</sub>—CH(OH)—CH<sub>2</sub>—O—D—O— group, in which D is C<sub>2</sub>-C<sub>10</sub>alkylene, C<sub>6</sub>-C<sub>15</sub>arylene, C<sub>6</sub>-C<sub>12</sub>cycloalkylene, or, if R<sup>13</sup> is not alkanoyl, alkenoyl or benzoyl, R<sup>14</sup> can also be a dibasic radical of an aliphatic, cycloaliphatic or aromatic dicarboxylic acid or dicarbamic acid or also the group —CO—, or when n is 1, R<sup>13</sup> and R<sup>14</sup> together can be the dibasic radical of an aliphatic, cycloaliphatic or aromatic 1,2- or 1,3-di-carboxylic acid.

Any C<sub>1</sub>-C<sub>12</sub>alkyl or C<sub>1</sub>-C<sub>18</sub>alkyl substituents present have the meaning already defined in a).

Any C<sub>5</sub>-C<sub>7</sub>cycloalkyl substituents present are particularly cyclohexyl.

As C<sub>7</sub>-C<sub>8</sub>aralkyl, R<sup>13</sup> is particularly phenylethyl or above all benzyl. As C<sub>2</sub>-C<sub>3</sub>hydroxyalkyl, R<sup>13</sup> is particularly 2-hydroxyethyl or 2-hydroxypropyl.

As C<sub>2</sub>-C<sub>18</sub>alkanoyl, R<sup>13</sup> is for example propionyl, butyryl, octanoyl, dodecanoyl, hexadecanoyl, octadecanoyl, but preferably acetyl, and as C<sub>3</sub>-C<sub>5</sub>alkenoyl, R<sup>13</sup> is particularly acryloyl.

As C<sub>2</sub>-C<sub>8</sub>alkenyl, R<sup>14</sup> is for example allyl, methallyl, 2-but enyl, 2-pentenyl, 2-hexenyl or 2-octenyl.

As C<sub>1</sub>-C<sub>4</sub>alkyl substituted by a hydroxyl, cyano, alkoxy carbonyl or carbamide group, R<sup>14</sup> can be, for example, 2-hydroxyethyl, 2-hydroxypropyl, 2-cyanoethyl, methoxycarbonylmethyl, 2-ethoxycarbonylethyl, 2-aminocarbonylpropyl or 2-(dimethylaminocarbonyl)ethyl.

Any C<sub>2</sub>-C<sub>12</sub>alkylene substituents present are, for example, ethylene, propylene, 2,2-dimethylpropylene, tetramethylene, hexamethylene, octamethylene, decamethylene or dodecamethylene.

Any C<sub>6</sub>-C<sub>15</sub>arylene substituents present are, for example, o-, m- or p-phenylene, 1,4-naphthylene or 4,4'-diphenylene.

As C<sub>6</sub>-C<sub>12</sub>cycloalkylene, D is especially cyclohexylene.

Preferred compounds of the formula V are those in which n is 1 or 2, R is hydrogen, R<sup>11</sup> is hydrogen or methyl, R<sup>13</sup> is hydrogen, C<sub>1</sub>-C<sub>12</sub>alkyl or a group of the formula



and when n=1, R<sup>14</sup> is hydrogen or C<sub>1</sub>-C<sub>12</sub>alkyl, and when n=2, R<sup>14</sup> is C<sub>2</sub>-C<sub>8</sub>alkylene.

Examples of polyalkylpiperidine compounds of this class are the following compounds:

- 37) N,N'-bis(2,2,6,6-tetramethylpiperidin-4-yl)hexamethylene-1,6-diamine  
 38) N,N'-bis(2,2,6,6-tetramethylpiperidin-4-yl)hexamethylene-1,6-diacetamide  
 39) bis(2,2,6,6-tetramethylpiperidin-4-yl)amine  
 40) 4-benzoylamino-2,2,6,6-tetramethylpiperidine  
 41) N,N'-bis(2,2,6,6-tetramethylpiperidin-4-yl)-N,N'-dibutyl adipamide  
 42) N,N'-bis(2,2,6,6-tetramethylpiperidin-4-yl)-N,N'-dicyclohexyl-2-hydroxypropylene-1,3-diamine

- 43) N,N'-bis(2,2,6,6-tetramethylpiperidin-4-yl)-p-xylylenediamine  
 44) N,N'-bis(2,2,6,6-tetramethylpiperidin-4-yl)succinamide  
 45) di(2,2,6,6-tetramethylpiperidin-4-yl) N-(2,2,6,6-tetramethylpiperidin-4-yl)-aminodipropionate  
 46) The compound of the formula



- 47) 4-(bis-2-hydroxyethylamino)-1,2,2,6,6-pentamethylpiperidine  
 48) 4-(3-methyl-4-hydroxy-5-tert-butylbenzoamido)-2,2,6,6-tetramethylpiperidine  
 49) 4-methacrylamido-1,2,2,6,6-pentamethylpiperidine  
 c) compounds of the formula (VI)



in which n is the integer 1 or 2, R and R<sup>11</sup> have the meaning defined in a), and when n is 1, R<sup>15</sup> is C<sub>2</sub>-C<sub>8</sub>alkylene or C<sub>2</sub>-C<sub>8</sub>hydroxyalkylene or C<sub>4</sub>-C<sub>22</sub>acyloxyalkylene, and when n is 2, R<sup>15</sup> is the group (—CH<sub>2</sub>)<sub>2</sub>C(CH<sub>2</sub>)<sub>2</sub>.

As C<sub>2</sub>-C<sub>8</sub>alkylene or C<sub>2</sub>-C<sub>8</sub>hydroxyalkylene, R<sup>15</sup> is for example ethylene, 1-methylethylene, propylene, 2-ethylpropylene or 2-ethyl-2-hydroxymethylpropylene.

As C<sub>4</sub>-C<sub>22</sub>acyloxyalkylene, R<sup>15</sup> is for example 2-ethyl-2-acetoxymethylpropylene.

Examples of polyalkylpiperidine compounds of this class are the following compounds:

- 50) 9-aza-8,8,10,10-tetramethyl-1,5-dioxaspiro[5.5]undecane  
 51) 9-aza-8,8,10,10-tetramethyl-3-ethyl-1,5-dioxaspiro[5.5]undecane  
 52) 8-aza-2,7,7,8,9,9-hexamethyl-1,4-dioxaspiro[4.5]decane

- 53) 9-aza-3-hydroxymethyl-3-ethyl-8,8,9,10,10-pentamethyl-1,5-dioxaspiro[5.5]undecane  
 54) 9-aza-3-ethyl-3-acetoxymethyl-9-acetyl-8,8,10,10-tetramethyl-1,5-dioxaspiro[5.5]undecane  
 55) 2,2,6,6-tetramethylpiperidine-4-spiro-2'-(1',3'-dioxan-5'-spiro-5''-(1'',3''-dioxan)-2''-spiro-4''-(2'',2'',6'',6''-tetramethylpiperidine).  
 d) compounds of the formulae VIIA, VIIB and VIIC



in which n is the integer 1 or 2, R and R<sup>11</sup> have the meaning defined in a), R<sup>16</sup> is hydrogen, C<sub>1</sub>-C<sub>12</sub>alkyl, allyl, benzyl, glycidyl or C<sub>2</sub>-C<sub>6</sub>alkoxyalkyl, and when n is 1, R<sup>17</sup> is hydrogen, C<sub>1</sub>-C<sub>12</sub>alkenyl, C<sub>7</sub>-C<sub>9</sub>aralkyl, C<sub>5</sub>-C<sub>7</sub>cycloalkyl, C<sub>2</sub>-C<sub>4</sub>hydroxyalkyl, C<sub>2</sub>-C<sub>6</sub>alkoxyalkyl, C<sub>6</sub>-C<sub>10</sub>aryl, glycidyl or a group of the formula —(CH<sub>2</sub>)<sub>p</sub>-COO—Q or the formula —(CH<sub>2</sub>)<sub>p</sub>-O—CO—Q, in which p is 1 or 2 and Q is C<sub>1</sub>-C<sub>4</sub>alkyl or phenyl, and when n is 2, R<sup>17</sup> is C<sub>2</sub>-C<sub>12</sub>alkylene, C<sub>4</sub>-C<sub>12</sub>alkenylene, C<sub>6</sub>-C<sub>12</sub>arylene, a group —CH<sub>2</sub>-CH(OH)—CH<sub>2</sub>—O—D—O—CH<sub>2</sub>—CH(OH)—CH<sub>2</sub>—, in which D is C<sub>2</sub>-C<sub>10</sub>alkylene, C<sub>6</sub>-C<sub>12</sub>arylene, C<sub>6</sub>-C<sub>12</sub>cycloalkylene or a group —CH<sub>2</sub>C(H(OZ')CH<sub>2</sub>—(OCH<sub>2</sub>CH(OZ')CH<sub>2</sub>)<sub>2</sub>—, in which Z' is hydrogen, C<sub>1</sub>-C<sub>12</sub>alkyl, allyl, benzyl, C<sub>2</sub>-C<sub>12</sub>alkanoyl or benzoyl, T<sub>1</sub> and T<sub>2</sub> independently of one another are hydrogen, C<sub>1</sub>-C<sub>12</sub>alkyl or C<sub>6</sub>-C<sub>10</sub>aryl or C<sub>7</sub>-C<sub>9</sub>aralkyl which are unsubstituted or substituted by halogen or C<sub>1</sub>-C<sub>4</sub>alkyl, or T<sub>1</sub> and T<sub>2</sub> together form with the carbon atom connecting them a C<sub>5</sub>-C<sub>12</sub>cycloalkane ring.

Any C<sub>1</sub>-C<sub>12</sub>alkyl substituents present are, for example, methyl, ethyl, n-propyl, n-butyl, sec-butyl, tert-butyl, n-hexyl, n-octyl, 2-ethylhexyl, n-nonyl, n-decyl, n-undecyl or n-dodecyl.

Any C<sub>1</sub>-C<sub>12</sub>alkyl substituents present can be, for example, the groups defined above and additionally also, for example, n-tridecyl, n-tetradecyl, n-hexadecyl or n-octadecyl.

Any C<sub>2</sub>-C<sub>6</sub>alkoxyalkyl substituents present are, for example, methoxymethyl, ethoxymethyl, propoxymethyl, tert-butoxymethyl, ethoxyethyl, ethoxypro-

pyl, n-butoxyethyl, tert-butoxyethyl, isopropoxyethyl or propoxypropyl.

As  $C_3$ - $C_5$ alkenyl,  $R^{17}$  is, for example, 1-propenyl, allyl, methallyl, 2-butenyl or 2-pentenyl.

As C<sub>7</sub>-C<sub>9</sub>aralkyl, R<sup>17</sup>, T<sub>1</sub> and T<sub>2</sub> are particularly phenethyl or above all benzyl. Any cycloalkane ring formed by T<sub>1</sub> and T<sub>2</sub> together with the carbon atom can be, for example, a cyclopentane, cyclohexane, cyclooctane or cyclododecane ring.

As C<sub>2</sub>-C<sub>4</sub>hydroxyalkyl, R<sup>17</sup> is, for example, 2-hydroxyethyl, 2-hydroxypropyl, 2-hydroxybutyl or 4-hydroxybutyl.

As  $C_6$ -C<sub>10</sub>aryl, R<sup>17</sup>, T<sub>1</sub> and T<sub>2</sub> are especially phenyl,  $\alpha$ - or  $\beta$ -naphthyl which are unsubstituted or substituted by halogen or C<sub>1</sub>-C<sub>4</sub>alkyl.

- 59) 3-glycidyl-1,3,8-triaza-7,7,8,9,9-pentamethyl-spiro[4.5]decane-2,4-dione

60) 1,3,7,7,8,9,9-heptamethyl-1,3,8-triazaspiro[4.5]decane-2,4-dione

5 61) 2-iso-propyl-7,7,9,9-tetramethyl-1-oxa-3,8-diaza-4-oxo-spiro[4.5]-decane

62) 2,2-dibutyl-7,7,9,9-tetramethyl-1-oxa-3,8-diaza-4-oxospiro[4.5]decane

63) 2,2,4,4-tetramethyl-7-oxa-3,20-diaza-21-oxodispiro[5.1.11.2]-heneicosane

10 64) 2-butyl-7,7,9,9-tetramethyl-1-oxa-4,8-diaza-3-oxospiro[4.5]decane

65) 8-acetyl-3-dodecyl-1,3,8-triaza-7,7,9,9-tetramethyl-spiro[4.5]decane-2,4-dione

15 or the compounds of the following formulae:

15 or the compounds of the following formulae:



As  $C_2-C_{12}$ alkylene,  $R^{17}$  is, for example, ethylene, propylene, 2,2-di-methylpropylene, tetramethylene, 50 hexamethylene, octamethylene, decamethylene or dodecamethylene.

As C<sub>4</sub>-C<sub>12</sub>alkenylene, R<sup>17</sup> is particularly 2-butenylene, 2-pentenylene or 3-hexenylene.

As  $C_6-C_{12}$ arylene,  $R^{17}$  is, for example, o-, m- or p- 55 phenylene, 1,4-naphthylene or 4,4'-diphenylene.

As  $C_2C_{12}$ alkanoyl,  $Z'$  is, for example, propionyl, butyryl, octanoyl, dodecanoyl, but preferably acetyl.

As  $C_2C_{10}$ alkylene,  $C_6-C_{15}$ arylene or  $C_6-C_{12}$ cy-cloalkylene, D has the meaning defined in b).

Examples of polyalkylpiperidine compounds of this class are the following compounds:

56) 3-benzyl-1,3,8-triaza-7,7,9,9-tetramethylspiro[4.5]-decan-2,4-dione

- 57) 3-n-octyl-1,3,8-triaza-7,7,9,9-tetramethylspiro[4.5]- 65  
 decane-2,4-dione  
 58) 3-allyl-1,3,8-triaza-1,7,7,9,9-pentamethylspiro[4.5]-  
 decane-2,4-dione

e) compounds of the formula VIII



in which  $n$  is the integer 1 or 2 and  $R^{18}$  is a group of the formula



in which R and R<sup>11</sup> have the meaning defined in a), E is —O— or —NR<sup>11</sup>—, A is C<sub>2</sub>—C<sub>6</sub>alkylene or —(CH<sub>2</sub>)<sub>3</sub>—O—, and x is the integers 0 or 1, R<sup>19</sup> is the same as R<sup>18</sup> or is one of the groups —NR<sup>21</sup>R<sup>22</sup>, —OR<sup>23</sup>, —NHCH<sub>2</sub>OR<sup>23</sup> or —N(CH<sub>2</sub>OR<sup>23</sup>)<sub>2</sub>, and when n is 1, R<sup>20</sup> is the same as R<sup>18</sup> or R<sup>19</sup>, and when n=2, R<sup>20</sup> is a group —E—B—E—, in which B is C<sub>2</sub>—C<sub>6</sub>alkylene which is uninterrupted or interrupted by —N(R<sup>21</sup>)—, R<sup>11</sup> is C<sub>1</sub>—C<sub>12</sub>alkyl, cyclohexyl, benzyl or C<sub>1</sub>—C<sub>4</sub>hydroxyalkyl or a group of the formula



R<sup>22</sup> is C<sub>1</sub>—C<sub>12</sub>alkyl, cyclohexyl, benzyl, C<sub>1</sub>—C<sub>4</sub>hydroxyalkyl, and R<sup>23</sup> is hydrogen, C<sub>1</sub>—C<sub>12</sub>alkyl or phenyl, or R<sup>21</sup> and R<sup>22</sup> together are C<sub>4</sub>—C<sub>5</sub>alkylene or C<sub>4</sub>—C<sub>5</sub>oxoalkylene, for example



5 or R<sup>21</sup> and R<sup>22</sup> in each case are also a group of the formula



20 Any C<sub>1</sub>—C<sub>12</sub>alkyl substituents present are, for example, methyl, ethyl, n-propyl, n-butyl, sec-butyl, tert-butyl, n-hexyl, n-octyl, 2-ethylhexyl, n-nonyl, n-decyl, n-undecyl or n-dodecyl.

25 Any C<sub>1</sub>—C<sub>4</sub>hydroxyalkyl substituents present are, for example, 2-hydroxyethyl, 2-hydroxypropyl, 3-hydroxypropyl, 2-hydroxybutyl or 4-hydroxybutyl.

C<sub>2</sub>—C<sub>6</sub>alkylene as A is, for example, ethylene, propylene, 2,2-dimethylpropylene, tetramethylene or hexamethylene.

C<sub>4</sub>—C<sub>5</sub>alkylene or C<sub>4</sub>—C<sub>5</sub>oxaalkylene as R<sup>21</sup> and R<sup>22</sup> together are, for example, tetramethylene, pentamethylene or 3-oxapentamethylene.

Examples of polyalkylpiperidine compounds of this class are the compounds of the following formulae:



70)



71)

• -continued



72)



73)



74)



75)

-continued



76)



77)



78)

-continued

79)



(80)



f) oligomers or polymeric compounds whose recurring structural unit comprises a 2,2,6,6-tetraalkylpiperidine radical of the formula (I), particularly polyesters, polyethers, polyamides, polyamines, polyurethanes, polyureas, polyaminotriazines, poly(meth)acrylates,

poly(meth)acrylamide and their copolymers which comprise such radicals.

Examples of 2,2,6,6-polyalkylpiperidine light stabilizers of this class are the compounds of the following formulae where  $m$  is an integer of 2 to about 200.



81)



82)



83)

-continued

84)



85)



86)



87)



88)



89)



-continued

90)



91)



92)



93)



94)

g) compounds of the formula IX

(IX) 60 in which R and R<sup>11</sup> have the meaning defined in a).  
 Preferred compounds of the formula IX are those in which R is hydrogen or methyl and R<sup>11</sup> is hydrogen or methyl.

Examples of such compounds are:

- 65 95) 2,2,6,6-tetramethyl-4-piperidone (triacetonamine)  
 96) 1,2,2,6,6-pentamethyl-4-piperidone  
 97) 2,2,6,6-tetramethyl-4-piperidone-1-oxyl  
 98) 2,3,6-trimethyl-2,6-diethyl-4-piperidone



The amount of (B) and (C) added to the base oil (A) depends on the type of the base oil and the desired degree of stabilization. Generally the total of (B) and (C) is 0.1 to 2% by weight, preferably 0.5 to 1% by weight, based on (A). The ratio of (B) to (C) can vary within wide limits; (B) is generally the quantitatively dominant component. The ratio (B):(C) is preferably 3-5:1.

The component (A) is a mineral or synthetic base oil, such as is normally used for the production of lubricants. Synthetic oils may be, for example, esters of polycarboxylic acids or of polyols; they may also be aliphatic polyesters or poly- $\alpha$ -olefins, silicones, phosphoric acid esters or polyalkylene glycols. The lubricant may also be a grease based on an oil and a thickener. Such lubricants are described, for example, in D. Klamann "Schmierstoffe und arverwandte Produkte" ["Lubricants and Related Products"], Verlag Chemie, Weinheim 1982.

The lubricant may additionally contain other additives, for example other antioxidants, metal passivators, rust inhibitors, viscosity index improvers, pour point depressants, dispersants, surfactants or antiwear additives.

#### EXAMPLES OF PHENOLIC ANTIOXIDANTS

##### 1. Alkylated monophenolics

2,6-di-tert-butyl-4-methylphenol, 2,6-di-tert-butylphenol, 2-tert-butyl-4,6-dimethylphenol, 2,6-di-tert-butyl-4-ethylphenol, 2,6-di-tert-butyl-4-n-butylphenol, 2,6-di-tert-butyl-4-iso-butylphenol, 2,6-dicyclopentyl-4-methylphenol, 2-( $\alpha$ -methylcyclohexyl)-4,6-dimethylphenol, 2,6-di-octadecyl-4-methylphenol, 2,4,6-tricyclohexylphenol, 2,6-di-tert-butyl-4-methoxymethylphenol, o-tert-butylphenol.

##### 2. Alkylated hydroquinones

2,6-di-tert-butyl-4-methoxyphenol, 2,5-di-tert-butylhydroquinone, 2,5-di-tert-amylhydroquinone, 2,6-diphenyl-4-octadecyloxyphenol.

##### 3. Hydroxylated thiodiphenyl ethers

2,2'-thio-bis(6-tert-butyl-4-methylphenol), 2,2'-thio-bis(4-octylphenol), 4,4'-thio-bis(6-tert-butyl-3-methylphenol), 4,4'-thio-bis(6-tert-butyl-2-methylphenol).

##### 4. Alkylidene bisphenols

2,2'-methylene-bis(6-tert-butyl-4-methylphenol), 2,2'-methylene-bis(6-tert-butyl-4-ethylphenol), 2,2'-methylene-bis[4-methyl-6-( $\alpha$ -methylcyclohexyl)phenol], 2,2'-methylene-bis(4-methyl-6-cyclohexylphenol), 2,2'-methylene-bis(6-nonyl-4-methylphenol), 2,2'-methylene-bis(4,6-di-tert-butylphenol), 2,2'-ethylidene-bis(4,6-di-tert-butylphenol), 2,2'-ethylidene-bis(6-tert-butyl-4-isobutylphenol or -5-isobutylphenol), 2,2'-methylene-bis[6-( $\alpha$ -methylbenzyl)-4-nonylphenol], 2,2'-methylene-bis[6-( $\alpha$ , $\alpha$ -dimethylbenzyl)-4-nonylphenol], 4,4'-methylene-bis(2,6-di-tert-butylphenol), 4,4'-methylene-bis(6-tert-butyl-2-methylphenol), 1,1-bis(5-tert-butyl-4-hydroxy-2-methylphenyl)butane, 2,6-di(3-tert-butyl-5-methyl-2-hydroxybenzyl)-4-methylphenol, 1,1,3-tris(5-tert-butyl-4-hydroxy-2-methylphenyl)-3-n-dodecylmercaptobutane, ethylene glycol bis[3,3-bis(3'-tert-butyl-4'-hydroxyphenyl)butyrate], bis(3-tert-butyl-4-hydroxy-5-methylphenyl)dicyclopentadiene, bis[2-(3'-tert-butyl-2'-hydroxy-5'-methylbenzyl)-6-tert-butyl-4-methylphenyl]terephthalate.

##### 5. Benzyl compounds

1,3,5-tris(3,5-di-tert-butyl-4-hydroxybenzyl)-2,4,6-trimethylbenzene, bis(3,5-di-tert-butyl-4-hydroxybenzyl)sulfide, isoocetyl 3,5-di-tert-butyl-4-hydroxybenzyl-

mercaptoacetate, bis(4-tert-butyl-3-hydroxy-2,6-dimethylbenzyl)dithiol terephthalate, 1,3,5-tris(3,5-di-tert-butyl-4-hydroxybenzyl) isocyanurate, 1,3,5-tris(4-tert-butyl-3-hydroxy-2,6-dimethylbenzyl) isocyanurate, di-octadecyl 3,5-di-tert-butyl-4-hydroxybenzylphosphonate, monoethyl 3,5-di-tert-butyl-4-hydroxybenzylphosphonate calcium salt.

##### 6. Acylaminophenols

4-hydroxylauranilide, 4-hydroxystearanilide, 2,4-bis-octylmercapto-6-(3,5-di-tert-butyl-4-hydroxyanilino)-s-triazine, octyl N-(3,5-di-tert-butyl-4-hydroxyphenyl)-carbamate.

7. Esters of  $\beta$ -(3,5-di-tert-butyl-4-hydroxyphenyl)-propionic acid with monohydric or polyhydric alcohols, for example with methanol, diethylene glycol, octadecanol, triethylene glycol, 1,6-hexanediol, pentaerythritol, neopentyl glycol, tris-hydroxyethyl isocyanurate, thiidiethylene glycol, bishydroxyethyloxalic acid diamide.

8. Esters of  $\beta$ -(5-tert-butyl-4-hydroxy-3-methylphenyl)propionic acid with monohydric or polyhydric alcohols, for example with methanol, diethylene glycol, octadecanol, triethylene glycol, 1,6-hexanediol, pentaerythritol, neopentyl glycol, tris-hydroxyethyl isocyanurate, thiidiethylene glycol, dihydroxyethyloxalic acid diamide.

9. Amides of  $\beta$ -(3,5-di-tert-butyl-4-hydroxyphenyl)-propionic acid for example N,N'-bis(3,5-di-tert-butyl-4-hydroxyphenylpropionyl)hexamethylenediamine, N,N'-bis(3,5-di-tert-butyl-4-hydroxyphenylpropionyl)-trimethylenediamine, N,N'-bis(3,5-di-tert-butyl-4-hydroxyphenylpropionyl)hydrazine.

Examples of other antioxidants:

35 aliphatic or aromatic phosphites, esters of thiadipropionic acid or of thiodiacetic acid, or salts of dithiocarbamide acid or dithiophosphoric acid.

Examples of metal deactivators for example for copper:

40 triazoles, benzotriazoles and their derivatives, toltriazoles and their derivatives, 2-mercaptopbenzothiazole, 2-mercaptopbenzotriazole, 2,5-dimercaptobenzotriazole, 2,5-dimercaptobenzothiadiazole, 5,5'-methylenebisbenzotriazole, 4,5,6,7-tetrahydrobenzotriazole, salicylidenepropylenediamine, salicylaminoguanidine and their salts.

Examples of rust inhibitors:

a) Organic acids and esters, metal salts and anhydrides thereof, for example: N-oleylsarcosine, sorbitol monooleate, lead naphthenate, alkenylsuccinic anhydride, for example dodecylsuccinic anhydride, alkenylsuccinic acid hemiesters and hemi-amides, and 4-nonylphenoxyacetic acid.

b) Nitrogenous compounds, for example:

I. primary, secondary or tertiary aliphatic or cycloaliphatic amines and amine salts of organic and inorganic acids, for example oil-soluble alkylammonium carboxylates.

II. heterocyclic compounds, for example: substituted imidazolines and oxazolines.

c) Phosphorus compounds, for example: amine salts of partial esters of phosphoric acid or partial esters of phosphonic acid, zinc dialkyldithiophosphates.

d) Sulfur compounds, for example: barium dinonylnaphthalenesulfonates, calcium petroleum sulfonates.

Examples of viscosity index improvers:

polyacrylates, polymethacrylates, vinylpyrrolidone-methacrylate copolymers, polyvinylpyrrolidones, poly-

butenes, olefin copolymers, styrene/acrylate copolymers, polyethers.

Examples of pour point depressants:

polymethacrylate, alkylated naphthalene derivatives.

Examples of dispersants/surfactants:

polybutenylsuccinamides or -imides, polybutenylphosphonic acid derivatives, basic magnesium, calcium and barium sulfonates and phenolates.

Examples of antiwear additives:

compounds containing sulfur and/or phosphorus and/or halogen, such as sulfurized vegetable oils, zinc dialkyldithiophosphates, tritolylphosphate, chlorinated paraffins, alkyl sulfides, aryl disulfides and aryl trisulfides, triphenylphosphorothionates, diethanolaminomethyltolyltriazole, di(2-ethylhexyl)aminomethyltolyltriazole.

The addition of phenolic antioxidants and/or of aliphatic and aromatic phosphites or phosphonites which are capable of increasing the stabilizing effect of the components (B) and (C), is particularly important.

Examples of suitable phosphites and phosphonites are: triphenyl phosphite, decyldiphenyl phosphite, phenyldidecyl phosphite, tris(nonylphenyl) phosphite, tri-lauryl phosphite, trioctadecyl phosphite, distearylpen-taerythritol diphosphite, tris(2,4-di-tert-butylphenyl) phosphite, diisodecylpentaerythritol diphosphite, bis(2,4-di-tert-butylphenyl)pentaerythritol diphosphite, tristearyl sorbitol triphosphite, tetrakis(2,4-d-tert-butylphenyl)-4,4'-biphenylene diphosphonite, bis(2,6-di-tert-butyl-4-methylphenyl)pentaerythritol diphosphite.

The individual additives are dissolved in the oil. To speed up the dissolution, the oil may be first heated or the additives may be first dissolved in a solvent.

The lubricant may also contain solid lubricant additives, for example graphite or molybdenum sulfide.

The examples below elucidate the invention in greater detail. The parts and percentages are parts and percentages by weight, unless stated otherwise.

#### EXAMPLE 1

The induction period of the oxidation of the oil samples by air containing 400 ppm of  $\text{NO}_2$  is determined under isothermal conditions using a differential scanning calorimeter (Du Pont Thermoanalyser 1090). The measurement is carried out at 170°C. at a pressure of 8 bar. A reference mineral oil (Aral 136) containing 1% by volume of 1-decene added in order to boost its susceptibility to oxidation, is used as the base oil. The following amine stabilizers are added to the oil.

Aromatic amines:

A-1 An industrial mixture produced by reacting diphenylamine with diisobutylene, comprising  
 a) 3% of diphenylamine  
 b) 14% of 4-tert-butylidiphenylamine,

55

- c) 30% of 4-tert-octylidiphenylamine, 4,4'-di-tert-butylidiphenylamine and 2,4,4'-tri-tert-butylidiphenylamine,  
 d) 29% of 4-tert-butyl-4'-tert-octylidiphenylamine, 2,2'- and 3,3'-di-tert-octylidiphenylamine and 2,4-di-tert-butyl-4'-tert-octylidiphenylamine,  
 e) 18% of 4,4'-di-tert-octylidiphenylamine,  
 f) 6% of 2,4-di-tert-octyl-4'-tert-butylidiphenylamine.

A-2 3,7-di-(tert-octyl)phenothiazine

Hindered amines:

- H-1 di(2,2,6,6-tetramethylpiperidin-4-yl) sebacate  
 H-2 2,2,6,6-tetramethyl-4-piperidone  
 H-3 di(2,2,6,6-tetramethylpiperidin-4-yl) succinate  
 H-4 di(1,2,2,6,6-pentamethylpiperidin-4-yl) sebacate  
 H-5 2,3,6-trimethyl-2,6-diethyl-piperidone  
 H-6 2,2,6,6-tetramethyl-4-butylaminopiperidine

Table 1 lists the induction periods. The higher the induction period, the greater is the antioxidative effect of the stabilizer additives.

20

TABLE 1

| Aromatic amine | Hindered amine | Induction period (min) |
|----------------|----------------|------------------------|
| —              | —              | 43                     |
| 0.55% of A-1   | —              | 80                     |
| 0.45% of A-1   | 0.10% of H-1   | 91.5                   |
| 0.45% of A-1   | 0.10% of H-2   | 91.5                   |
| 0.45% of A-1   | 0.10% of H-3   | 90.05                  |
| 0.45% of A-1   | 0.10% of H-4   | 90                     |
| 0.45% of A-1   | 0.10% of H-5   | 84.5                   |
| 0.45% of A-1   | 0.10% of H-6   | 89                     |

30

#### EXAMPLE 2

Oxidation of hydrocarbons gives rise to oxygen-containing groups, for example hydroxyl, carboxyl or ester groups. Infra-red spectroscopy allows the amount of such groups to be measured and to determine therefrom the effect of the antioxidants. For this purpose samples of a reference mineral oil (Aral® 136) containing 1% by volume of 1-decene added in order to boost its susceptibility to oxidation, is heated under isothermal conditions in air containing 400 ppm of  $\text{NO}_2$ , for 12 hours at a pressure of 8 bar. The IR absorption at  $1730\text{ cm}^{-1}$  and  $1630\text{ cm}^{-1}$  is then determined. The greater these values, the greater is the effect of the stabilizers. Tables 2a and 2b demonstrate the results at various temperatures.

40

TABLE 2a

| Stabilizer                  | IR Absorption            |                          |
|-----------------------------|--------------------------|--------------------------|
|                             | at $1730\text{ cm}^{-1}$ | at $1630\text{ cm}^{-1}$ |
| 0.55% of A-1                | 0.471                    | 1.051                    |
| 0.45% of A-1 + 0.10% of H-2 | 0.392                    | 0.839                    |
| 0.45% of A-1 + 0.10% of H-3 | 0.424                    | 0.863                    |
| 0.45% of A-1 + 0.10% of H-5 | 0.396                    | 0.673                    |

50

TABLE 2b

Oxidation at  $150^\circ\text{ C}$ .

| Stabilizer                                        | IR Absorption            |                          |
|---------------------------------------------------|--------------------------|--------------------------|
|                                                   | at $1730\text{ cm}^{-1}$ | at $1630\text{ cm}^{-1}$ |
| 0.55% of A-1                                      | 0.557                    | 1.851                    |
| 0.45% of A-1 + 0.10% of H-4                       | 0.353                    | 1.500                    |
| 0.65% of A-1                                      | 0.384                    | 1.599                    |
| 0.45% of A-1 + 0.10% of H-4 + 0.10% of phenol B*) | 0.330                    | 1.279                    |
| 0.45% of A-1 + 0.10% of A-2 +                     | 0.340                    | 1.443                    |

TABLE 2b-continued

| Stabilizer   | IR Absorption            |                          |
|--------------|--------------------------|--------------------------|
|              | at 1730 cm <sup>-1</sup> | at 1630 cm <sup>-1</sup> |
| 0.10% of H-4 |                          |                          |

\*) phenol B = compound of the formula



### EXAMPLE 3

The oxidation characteristics of the lubricating oils stabilized according to the invention were also tested by the TOST (turbine oxidation stability test) method according to ASTM D-943. For this purpose 60 ml of water are added to 300 ml of a mineral oil (Mobil STOC K 305) and the oil is heated in the presence of iron or copper wire at 95° C. for 1000 hours, while oxygen is passed through. The measured parameters are formation of acids by determining the neutralization value TAN (mg of KOH/g of oil) and the amount of sludge formed.

For the stabilization either the amine A-1 is used on its own or in admixture with the hindered amine H-7 (2,2,6,6-tetramethyl-4-dodecyloxy-piperidine), the total concentration of the stabilizers being always 0.25%, based on the oil.

| A-1  | H-7 | TAN (mg KOH/g of oil) | Sludge (mg) |
|------|-----|-----------------------|-------------|
| 100% | —   | 0.46                  | 30          |
| 95%  | 5%  | 0.38                  | 27          |
| 90%  | 10% | 0.30                  | 24          |
| 75%  | 25% | 0.31                  | 27          |

### EXAMPLE 4

By analogy with Example 1, the induction period of the oxidation is measured at 170° C. For this purpose the following hindered amines are used:

H-8 N,N'-bis(2,2,6,6-tetramethylpiperidin-4-yl)hexamethylenediamine

H-9 N,N'-bis(2,2,6,6-tetramethylpiperidin-4-yl)pentamethylenediamine

H-10 4-(methoxypropylamino)-2,2,6,6-tetramethylpiperidine

TABLE 4

| Aromatic amine | Hindered amine | Induction period (min) |
|----------------|----------------|------------------------|
| —              | —              | 48                     |
| 0.55% of A-1   | —              | 86                     |
| 0.45% of A-1   | 0.10% of H-8   | 95                     |
| 0.45% of A-1   | 0.10% of H-9   | 96                     |
| 0.45% of A-1   | 0.10% of H-10  | 89                     |

### EXAMPLE 5

The induction period of the oxidation is determined at 170° C. as described in Example 1. The following aromatic amine is used for this purpose:

A-3 N-(p-octylphenyl)-1-naphthylamine

TABLE 5

| Aromatic amine | Hindered amine | Induction period (min) |
|----------------|----------------|------------------------|
| 0.55% of A-3   | —              | 52.8                   |
| 0.45% of A-3   | 0.10% of H-7   | 66                     |

### EXAMPLE 6

Oxidation resistance can be also determined by measuring the viscosity increase when the oil is treated with oxygen at elevated temperature.

For this purpose a stream of oxygen (1 liter/h) is passed through the oil at 150° C. for 70 hours. The susceptibility of the oil to oxidation is first boosted by the addition of a catalytic amount of copper naphthenate. The viscosity of the oil is measured before and after the oxidation using an Ubbelohde viscometer.

TABLE 6

| Oil                                              | Percentage viscosity increase |
|--------------------------------------------------|-------------------------------|
| base oil                                         | 168%                          |
| base oil containing 0.6% of A-1 and 0.15% of H-8 | 3.4%                          |

We claim:

1. A lubricant composition which comprises
  - (A) a mineral or synthetic base oil or a mixture of such oils;
  - (B) at least one aromatic amine of formula II



in which

R<sup>3</sup> is hydrogen, C<sub>1</sub>-C<sub>12</sub>alkyl, benzyl, allyl, methallyl, phenyl or a group —CH<sub>2</sub>SR<sup>4</sup>,

R<sup>4</sup> is C<sub>4</sub>-C<sub>18</sub>alkyl, —CH<sub>2</sub>COO(C<sub>4</sub>-C<sub>18</sub>alkyl), or —CH<sub>2</sub>CH<sub>2</sub>COO(C<sub>4</sub>-C<sub>18</sub>alkyl), and

R<sup>5</sup> and R<sup>6</sup> independently of one another are hydrogen, C<sub>1</sub>-C<sub>18</sub>alkyl or C<sub>7</sub>-C<sub>9</sub>phenylalkyl; and

(C) at least one compound of formula IV, V or IX



in which

R is hydrogen,

R<sup>11</sup> is hydrogen or methyl,

n is 2, and

R<sup>12</sup> is a diacyl radical of an aliphatic dicarboxylic acid having 4 to 12 carbon atoms; or



in which

n is 1 or 2,

R is hydrogen,

R<sup>11</sup> is hydrogen or methyl,

R<sup>13</sup> is hydrogen, C<sub>1</sub>-C<sub>12</sub>alkyl or a group of the formula

(IV) 5

10

and, when n is 1, R<sup>14</sup> is hydrogen or C<sub>1</sub>-C<sub>12</sub>alkyl, and when n is 2, R<sup>14</sup> is C<sub>2</sub>-C<sub>8</sub>alkylene; or



15



20

in which

R is hydrogen, and

R<sup>11</sup> is hydrogen or methyl.

25 2. The composition according to claim 1 which comprises as the component (B) at least one compound of the formula II, in which R<sup>3</sup> is hydrogen, C<sub>1</sub>-C<sub>8</sub>alkyl, benzyl, allyl or a group —CH<sub>2</sub>SR<sup>4</sup>, R<sup>4</sup> is C<sub>8</sub>-C<sub>18</sub>alkyl or —CH<sub>2</sub>COO(C<sub>8</sub>-C<sub>18</sub>alkyl), and R<sup>5</sup> and R<sup>6</sup> independently of one another are H, C<sub>1</sub>-C<sub>12</sub>alkyl or C<sub>7</sub>-C<sub>9</sub>phenylalkyl.

30 3. The composition according to claim 1 which comprises as the component (B) at least one compound of the formula (II), in which R<sup>3</sup> is hydrogen and R<sup>5</sup> and R<sup>6</sup> independently of one another are H or C<sub>4</sub>-C<sub>12</sub>alkyl.

35 4. The composition according to claim 1 which comprises as the component (B) 3,7-di-tert-octylphenothiazine.

40 5. The composition according to claim 1 which comprises 0.1 to 2% by weight of the total of (B) and (C), based on (A).

45 6. The composition according to claim 1 wherein the ratio of (B) to (C) is 3-5 parts by weight of (B) per part by weight of (C).

7. The composition according to claim 1 which additionally contains a phenolic antioxidant (D).

8. The composition according to claim 1 which additionally contains an aliphatic or aromatic phosphite or phosphonite (E).

50 \* \* \* \* \*

55

60

65